# EUROPEAN PATENT SPECIFICATION

(11) **EP 3 355 319 B1**
(45) Date of publication and mention of the grant of the patent: **23.02.2022**
(21) Application number: 16874635.2
(22) Date of filing: 13.10.2016
(51) Int. Cl.: H01F 1/057, H01F 41/02, B22F 3/02, B22F 3/10

(54) **CORROSION-RESISTANT SINTERED NEODYMIUM-IRON-BORON MAGNET RICH IN LANTHANUM AND CERIUM, AND MANUFACTURING METHOD**
KORROSIONSBESTÄNDIGER GESINTERTER NEODYM-EISEN-BOR-MAGNET MIT HOHEM LANTHAN- UND CER-GEHALT SOWIE HERSTELLUNGSVERFAHREN
AIMANT NÉODYME-FER-BORE FRITTÉ RÉSISTANT À LA CORROSION RICHE EN LANTHANE ET EN CÉRIUM, ET PROCÉDÉ DE FABRICATION

(30) Priority: 16.12.2015 CN 201510943615
(43) Date of publication of application: 01.08.2018
(73) Proprietor: Zhejiang Dongyang Dmegc Rare Earth Magnet Co., Ltd, Dongyang, Zhejiang 322118 (CN)
(72) Inventor: LI, Runfeng, Dongyang Zhejiang 322118 (CN); CHEN, Qiaoling, Dongyang Zhejiang 322118 (CN)
(74) Representative: Elzaburu S.L.P.
(86) International application number: PCT/CN2016/101950
(87) International publication number: WO 2017/101577

(56) References cited:
- EP-A2- 0 187 538
- CN-A- 101 958 171
- CN-A- 102 220 538
- CN-A- 102 280 240
- CN-A- 102 347 126
- CN-A- 103 824 668
- CN-A- 105 427 994
- DE-A1-102015 105 764
- US-A1- 2015 248 954

## Description

### Technical Field

The present application relates to the technical field of neodymium-iron-boron (NdFeB) magnets rich in lanthanum and/or cerium, and more particularly relates to a corrosion-resistant sintered NdFeB magnet rich in lanthanum and/or cerium and a manufacturing method.

### Background Art

An NdFeB-based rare earth permanent magnet material is a third-generation rare earth permanent magnet functional material invented in the early 1980s, which has excellent magnetic properties of high remanence, high coercivity and high magnetic energy product, is thus widely used in automation technology, communication and transportation technology, information technology, aerospace technology and other sectors of the national economy, and becomes one of important basic materials supporting the contemporary electronic information industry. By this year, the usage has reached 100,000 tons, and the material has become an important material basis of modern science and technology and people's livelihood.

With the improvement of material usage, the amount of rare earth materials used as a main raw material for material manufacturing is continuously increasing. More importantly, the application field of rare earth materials as "vitamins" of modern industry is not limited to the production of rare earth permanent magnet materials. For example, in recent years, manufacturers of sintered NdFeB permanent magnet materials use relatively low-priced rare earth gadolinium element to partially replace more expensive rare earth praseodymium and neodymium elements to produce low-cost sintered NdFeB magnets, but the important application field of gadolinium is in the field of magnetic refrigeration materials and optical information storage sectors, so it is a waste of manufacturing low-cost sintered NdFeB permanent magnets with gadolinium instead of neodymium in a strict sense. Once gadolinium is found to have more important application, irreparable loss will be caused. Partial replacement of neodymium with holmium also has the same result and problem.

In the prior art, the two rare earth elements Pr and Nd are the main raw materials for producing sintered NdFeB rare earth permanent magnet materials, and the average use amount in materials is about 19 wt% to 33 wt%. However, in order to obtain some high-coercivity magnet materials, a small amount of Dy and Tb heavy rare earth elements and other non-rare earth metals such as Nb, Cu, Al, Ga, Ti, V, Mn, Zn, Zr, W, Si, Sn, Cr and Mo also need to be properly added to compose the ratio of the entire material. In the current domestic manufacturing level of sintered NdFeB permanent magnet materials, the mass production of medium and low grade products with Hcj less than or equal to 17kOe no longer needs to add Dy, Tb and other heavy rare earth elements, but the dependence on Pr and Nd as two kinds of light rare earth elements is increasingly prominent. The two elements Pr and Nd only account for 6 to 7wt% content in rare earth minerals. In order to meet the production of sintered NdFeB permanent magnet materials rich in lanthanum and/or cerium, the exploitation of rare earth resources is bound to be accelerated, causing the generation of more high-peak rare earth waste ore rich in lanthanum and/or cerium, thus increasing environmental pollution.

Therefore, if lanthanum cerium rare earth elements can be used to partially replace praseodymium neodymium materials for manufacturing NdFeB rare earth permanent magnet materials, the cost of materials can be reduced and a balanced use effect of resources can be achieved. However, due to easier oxidation of lanthanum and cerium elements than praseodymium and neodymium, the sintered NdFeB permanent magnet material with added lanthanum and cerium elements has worse corrosion resistance. Even if plated with some metal coating and placed in the air, a magnet will be severely corroded half a year later, with almost no practical value.

Based on these reasons, the improvement of the corrosion resistance of sintered NdFeB materials rich in lanthanum and/or cerium per se has become the basis of the material having practical value. The main reason for the corrosion of an NdFeB magnet lies in the electrode potential difference between a main phase and a phase rich in neodymium, in which the electrode potential of the main phase is higher than the electrode potential of the phase rich in neodymium, so that the phase rich in neodymium becomes an anode in the "galvanic reaction" to accelerate the corrosion of the phase rich in neodymium, resulting in continuous intergranular corrosion of crystal grains in the magnet. The main phase is exfoliated and pulverized due to the loss of a grain boundary phase, so as to complete the macroscopic oxidation of the permanent magnet. Therefore, how to reduce the potential difference between two phases in a sintered NdFeB magnet is the key to improve the corrosion resistance of the magnet.

In order to counteract this mechanism, people add elements Co and Cu to a material to increase the corrosion resistance of sintered Nd-Fe-B materials, wherein element Cu is added as a small metal in an amount that is not excessive (0.05 wt% to 0.25 wt%), and element Cu forms a mass phase at a grain boundary of the magnet, and generally does not participate in the replacement of a main phase element, so an effect on the magnetic property is little. However, Co element will be distributed in the grain boundary of the magnet, and can replace Fe element to form an Nd₂Co₁₄B phase, thereby reducing the magnetic property of the material.

DE 10 2015 105764 A1 discloses a sintered magnet formed by mixing an R₂T₁₄B main phase alloy with a Ce-rich grain boundary phase alloy including Ce to replace for expensive Dy element. US 2015/248954 A1 discloses a sintered magnet formed by mixing two R₂T₁₄B alloys both inluding Ce, Co and Fe. CN 102 220 538 A discloses a sintered magnet formed by mixing an R₂T₁₄B first alloy mixed with a Co, Fe, Ce, La-containing second alloy.

### Summary of the Invention

In order to overcome the above defects in the prior art, the present invention provides a corrosion-resistant sintered NdFeB magnet rich in lanthanum and/or cerium and a manufacturing method, which can improve the corrosion resistance of the magnet based on ensuring the magnetic property of the magnet.

In order to achieve the above object, the present invention adopts the following technical schemes:
A corrosion-resistant sintered NdFeB magnet rich in lanthanum and/or cerium comprises an NdFeB rare earth permanent magnet material rich in lanthanum and/or cerium and an alloy material rich in Co for improving corrosion resistance of the material, wherein components of the NdFeB rare earth permanent magnetic material rich in lanthanum and/or cerium are Re_{α}Fe_{100-α-β-γ}B_{β}M_{γ}, in which Re is a rare earth element, including two or more than two elements selected from La, Ce and Nd, and inevitably containing Nd element; M is an additive element, including one or more than one element selected from Ti, V, Cr, Ni, Zn, Ga, Ge, Al, Zr, Nb, Co, Cu, Ag, Sn, W, Pb, Bi and Pd; Fe is Fe and unavoidable impurities; α, β and γ are the atomic percentage contents of the elements, wherein 12≤α≤17, 5.1≤β≤6.8, and 0.1≤γ≤7.8; the alloy material rich in Co includes two or more than two elements selected from Pr, Nd, Gd, Ho, Co, Ti, V, Zn, Ga, Al, Zr, Nb, Cu, Ag, Sn, Pb and Pd, and inevitably contains Co.

The present invention applies an alloy material rich in cobalt for improving the corrosion resistance of a material to doping and modifying an NdFeB rare earth permanent magnet material rich in lanthanum and/or cerium, so that more Co element in the sintered NdFeB magnet can be distributed on a grain boundary instead of forming an Nd₂Co₁₄B phase that affects the magnetic property of the magnet, which is conducive to the preservation of the magnetic property of the material and the improvement of the corrosion resistance of the grain boundary of the magnet.

Preferably, La and Ce elements in the rare-earth element Re account for 15 wt% to 45 wt% of the total use amounts of rare earth in the NdFeB rare earth permanent magnet material rich in lanthanum and/or cerium. The use of lanthanum and cerium light rare earth elements instead of praseodymium and neodymium rare earth elements will slow down the exploitation of rare earth resources and reduce the generation of high-peak rear earth waste ore rich in lanthanum and/or cerium, so as to reduce environmental pollution.

Preferably, the rare earth element Re further comprises one or more than one element selected from Pr, Pm, Sm, Eu, Gd, Ho, Er, Tm, Yb, Lu, Y and Sc.

Preferably, the alloy material rich in Co inevitably does not contain element Fe to improve the corrosion resistance of the grain boundary of the magnet.

The present invention also provides a manufacturing method of a corrosion-resistant sintered NdFeB magnet rich in lanthanum and/or cerium, which comprises the following specific operation steps:
(1) Preparing an NdFeB rare earth permanent magnet material alloy rich in lanthanum and/or cerium according to components of an NdFeB rare earth permanent magnet material rich in lanthanum and/or cerium;
(2) Preparing an alloy material rich in Co according to components of the alloy material rich in Co;
(3) Breaking the NdFeB rare earth permanent magnet material alloy rich in lanthanum and/or cerium to obtain NdFeB rare earth permanent magnet material alloy powder rich in lanthanum and/or cerium with an average particle size of 2.5 to 4.5µm;
(4) Adding the alloy material rich in Co obtained in step (2) into the NdFeB rare earth permanent magnet material alloy powder rich in lanthanum and/or cerium according to a certain mass percentage content, wherein a process of pulverizing and mixing the alloy material rich in Co makes the alloy material rich in Co to be uniformly mixed into the NdFeB rare earth permanent magnet alloy powder rich in lanthanum and/or cerium;
(5) Pressing and molding the mixed alloy powder into a blank in an oriented magnetic field ≥ 1.5T under the protection of a nitrogen atmosphere;
(6) Placing the molded blank in a high-vacuum sintering furnace for high-temperature sintering, and performing a two-stage tempering process to obtain the corrosion-resistant sintered NdFeB magnet rich in lanthanum and/or cerium.

After the above process, the prepared corrosion-resistant sintered NdFeB magnet rich in lanthanum and/or cerium will be composed of a phase rich in Nd, a main phase (Nd₂Fe₁₄B), alloy powder rich in Co and a very small amount of phase rich in B (Nd_{1.1}Fe₄B₄). The alloy powder rich in Co exists between gaps of main phase particles.

Preferably, a preparation process adopted in step (1) and step (2) is a casting process or a quick-setting sheet process; and in step (3), a breaking method adopted is mechanical breaking or hydrogen breaking plus jet milling.

Preferably, the preparation process adopted in step (1) and step (2) is a quick-setting sheet process.

Preferably, a roller speed of a cooling copper roller used in the quick-setting sheet process of step (2) is 5 to 15 times of a roller speed of a cooling copper roller used in the quick-setting sheet process of step (1), wherein 5 to 15 times of the roll speed is a preferred solution, and in step (2) preparation can also be performed at the same roll speed as that in step (1).

Preferably, in step (4), the mass percentage content of the alloy material rich in Co in the NdFeB rare earth permanent magnet material alloy rich in lanthanum and/or cerium is 1% to 5%.

Preferably, in step (6), sintering temperature is 1030 °C to 1090 °C and sintering time is 2.0 to 8.0 hours. The two-stage tempering process is that first tempering is carried out at 890 °C to 920 °C and constant temperature time is 1.5 to 3 hours; and secondary tempering is carried out at 480 °C to 520 °C and constant temperature time is 2 to 6 hours. Since the main phase has a melting point of about 1185 °C and the alloy powder rich in Co generally begins to melt at 600 °C to 750 °C, the NdFeB alloy in a sintering temperature state is composed of a solid main phase, a molten phase rich in Nd, a molten phase rich in B and a molten alloy phase rich in Co, and the molten phases permeate into gaps between solid powder particles of the main phase through methods of liquid-phase flow and molecular thermal movement, so that the alloy phase rich in Co better penetrates to the grain boundary in the main phase.

The corrosion-resistant sintered NdFeB magnet has the beneficial effects that the Co element in the magnet is more distributed on the grain boundary of the magnet through the innovation of the manufacturing method, the corrosion resistance of the magnet is improved on the basis of ensuring the magnetic property of the magnet, and the sintered NdFeB magnet rich in lanthanum and/or cerium has good corrosion resistance the same as that of an ordinary sintered NdFeB permanent magnet and becomes a rare earth permanent magnet material with practical application value.

### Detailed Description of the Invention

The present invention is further described below with reference to specific embodiments.

### Embodiment 1:

1, An NdFeB rare earth permanent magnet material rich in lanthanum and/or cerium and with components of Nd_{12.3}Ce_{2.4}Fe_{remaining}B_{6.0}M_{1.7} (at%) is prepared into an NdFeB rare earth permanent magnet material alloy rich in lanthanum and/or cerium by a quick-setting sheet process according to a technical scheme of the present invention;
2, An alloy material rich in Co and with components of Nd_{21.72}Pr_{7.41}Co_{70.87} (at%) is prepared by the quick-setting sheet process;
3, The alloy material rich in Co is added into the NdFeB rare earth permanent magnet material alloy rich in lanthanum and/or cerium at a ratio of 1 wt% for hydrogen breakage, and mixed alloy powder with an average particle diameter of 3.5 µm is obtained by a jet milling process;
4, The mixed alloy powder is pressed and molded to form a square blank of 52 ^{∗} 52 ^{∗} 29 (mm) in an orientation magnetic field ≥1.5T;
5, The molded blank is placed in a high-vacuum sintering furnace for sintering at 1035 °C for 6.0 hours, first tempering at 920 °C for two hours and secondary tempering at 500 °C for 3.5 hours to obtain a corrosion-resistant sintered NdFeB magnet rich in lanthanum and/or cerium.
6, The obtained Nd_{12.3}Ce_{2.4}Fe_{remaining}B_{6.0}M_{1.7} (at%) NdFeB rare earth permanent magnet alloy rich in lanthanum and/or cerium is directly prepared into a sintered NdFeB magnet rich in lanthanum and/or cerium without adding an alloy material rich in Co by using the same manufacturing process.

The two magnets are machined to obtain Φ10 ^{∗} 10 (mm) standard samples, and HAST experiments (131 °C, 96% RH, 2.6bar, 96H) are then conducted to test the corrosion resistance of the materials. The performance of the materials is shown as Table 1.

**Table 1 Corrosion resistance test results**

| Material components (at%, see the components in Embodiment 1) | Mass loss (mg/cm²) |
|---|---|
| Sintered NdFeB magnet rich in lanthanum and/or cerium | 52.36 |
| Sintered NdFeB magnet rich in lanthanum and/or cerium with addition of 1 wt% of alloy material rich in Co | 0.42 |

### Embodiment 2:

1, An NdFeB rare earth permanent magnet material rich in lanthanum and/or cerium and with components of Pr_{3.06}Nd_{8.96}Ce_{3.31}Fe_{remaining}B_{5.88}M_{2.25} (at%) is prepared into an NdFeB rare earth permanent magnet material alloy rich in lanthanum and/or cerium by a quick-setting sheet process according to the technical scheme of the present invention;
2, An alloy material rich in Co and with components of Nd_{23.41}Pr_{10.97}Co_{64.24}Zr_{1.38} (at%) is prepared by the quick-setting sheet process;
3, The NdFeB rare earth permanent magnet material alloy rich in lanthanum and/or cerium and the alloy material rich in Co are respectively subjected to hydrogen breaking, in any one period of a jet milling powder prepration process on the NdFeB rare earth permanent magnet material alloy rich in lanthanum and/or cerium, the alloy material rich in Co is added at a ratio of 2wt%, mixed alloy powder having an average particle diameter of 2.8 - 3.0 µm is obtained by powder prepration, and the mixed alloy powder is uniformly mixed by a mixer;
4, The uniformly mixed alloy powder is pressed and molded to form a square blank of 52 ^{∗} 52 ^{∗} 29 (mm) in an orientation magnetic field ≥1.8T;
5, The blank is placed into a high-vacuum sintering furnace for sintering at 1075 °C for 4.0 hours, first tempering at 890 °C for 1.5 hours and secondary tempering at 510 °C for 6.0 hours to obtain a sintered NdFeB magnet rich in lanthanum and/or cerium.
6, The obtained Pr3.06Nd8.96Ce3.31Fe remaining B5.88M2.25 (at%) NdFeB rare earth permanent magnet alloy rich in lanthanum and/or cerium is directly prepared into a sintered NdFeB magnet rich in lanthanum and/or cerium without adding the alloy material rich in Co by using the same manufacturing process.

The two magnets are machined to prepare Φ10 ^{∗} 10 (mm) standard samples, and HAST experiments (131 °C, 96% RH, 2.6bar, 96H) are then performed to test the corrosion resistance of the materials. The performance of the materials is shown as Table 2.

**Table 2 Corrosion resistance test results**

| Material components (at%, see the components in Embodiment 2) | Mass loss (mg/cm²) |
|---|---|
| Sintered NdFeB magnet rich in lanthanum and/or cerium | 78.25 |
| Sintered NdFeB magnet rich in lanthanum and/or cerium with addition of 2 wt% of alloy material rich in Co | 0.88 |

### Embodiment 3:

1, An NdFeB rare earth permanent magnet material rich in lanthanum and/or cerium and with components of Pr_{2.11}Nd_{6.18}Ce_{4.71}Gd_{0.84}Ho_{0.6}Fe_{remaining} B_{5.87}M_{1.08} (at%) is prepared into an NdFeB rare earth permanent magnet material alloy rich in lanthanum and/or cerium by a quick-setting sheet process according to the technical scheme of the present invention;
2, An alloy material rich in Co and with components of Nd_{36.98}Pr_{12.62}Co_{34.47}Cr_{1.95}Cu_{3.20}Zn_{1.55}Al_{3.76}Nb_{5.47} (at%) is prepared by the quick-setting sheet process;
3, The NdFeB rare earth permanent magnet material alloy rich in lanthanum and/or cerium and the alloy material rich in Co are respectively subjected to hydrogen breaking, and the NdFeB rare earth permanent magnet alloy is subjected to jet milling powder preparation to obtain permanent magnet alloy powder having an average particle diameter of 3.0 to 3.2 µm; the alloy material rich in Co is subjected to jet milling powder preparation to obtain alloy powder rich in Co and having an average particle diameter of 4.2 to 4.5 µm, the alloy powder rich in Co is added into the NdFeB rare earth permanent magnet material alloy powder rich in lanthanum and/or cerium at a ratio of 3wt%, and the two types of alloy powder are mixed uniformly by mixing;
4, The uniformly mixed powder is pressed and molded to form a square blank of 52 ^{∗} 52 ^{∗} 29 (mm) in an orientation magnetic field ≥2.2T;
5, The blank is placed into a high-vacuum sintering furnace for sintering at 1060 °C for 8.0 hours, first tempering at 910 °C for 3.0 hours and secondary tempering at 480 °C for 2.0 hours to obtain a sintered NdFeB magnet rich in lanthanum and/or cerium.
6, The obtained Pr_{2.11}N_{d6.18}Ce_{4.71}Gd_{0.84}Ho_{0.6}Fe_{remaining}B_{5.87}M_{1.08} (at%) NdFeB rare earth permanent magnet material alloy rich in lanthanum and/or cerium is directly prepared into a sintered NdFeB magnet without adding the alloy material rich in Co by using the same manufacturing process.

The two magnets are machined to prepare Φ10 ^{∗} 10 (mm) standard samples, and HAST experiments (131 °C, 96% RH, 2.6bar, 96H) are then performed to test the corrosion resistance of the materials. The performance of the materials is shown as Table 3.

**Table 3 Corrosion resistance test results**

| Material components (at%, see the components in Embodiment 3) | Mass loss (mg/cm²) |
|---|---|
| Sintered NdFeB magnet rich in lanthanum and/or cerium | 88.25 |
| Sintered NdFeB magnet rich in lanthanum and/or cerium with addition of 3 wt% of alloy material rich in Co | 0.78 |

### Embodiment 4:

1, An NdFeB rare earth permanent magnet material rich in lanthanum and/or cerium and with components of Nd_{7.34}Ce_{5.53}Gd_{0.41}Fe_{remaining}B_{5.91}M_{3.32} (at%) is prepared into an NdFeB rare earth permanent magnet material alloy rich in lanthanum and/or cerium by a quick-setting sheet process according to the technical scheme of the present invention;
2, An alloy material rich in Co and with components of Nd_{77.91}Pr_{10.71}Co_{11.38} (at%) is prepared by the quick-setting sheet process;
3, The NdFeB rare earth permanent magnet material alloy rich in lanthanum and/or cerium and the alloy material rich in Co are subjected to hydrogen breaking, the NdFeB rare earth permanent magnet material alloy rich in lanthanum and/or cerium is subjected to jet milling powder preparation to obtain NdFeB rare earth permanent magnet material alloy powder rich in lanthanum and/or cerium and having an average particle diameter of 3.4 to 3.6 µm, after powder preparation on the NdFeB rare earth permanent magnet material alloy rich in lanthanum and/or cerium, the alloy material rich in Co is added into a jet mill at a ratio of 4wt% for continuous powder preparation to obtain alloy powder rich in Co having an average particle diameter of 2.5 to 2.7 µm, the alloy powder rich in Co and the NdFeB rare earth permanent magnet material alloy powder are together contained into a barrel, and the two types of alloy powder are mixed uniformly by a three-dimensional mixer;
4, The uniformly mixed powder is pressed and molded to form a square blank of 52 ^{∗} 52 ^{∗} 29 (mm) in an orientation magnetic field ≥1.5T;
5, The blank is placed into a high-vacuum sintering furnace for sintering at 1060 °C for 3.5 hours, first tempering at 900 °C for 2.0 hours and secondary tempering at 510 °C for 3.5 hours to obtain a sintered NdFeB magnet rich in lanthanum and/or cerium.
6, The obtained Nd_{7.34}Ce_{5.53}Gd_{0.41}Fe_{remaining} B_{5.91}M_{3.32} (at%) NdFeB rare earth permanent magnet material alloy rich in lanthanum and/or cerium is directly prepared into a sintered NdFeB magnet rich in lanthanum and/or cerium without adding the alloy material rich in Co by using the same manufacturing process.

The two magnets are machined to prepare Φ10 ^{∗} 10 (mm) standard samples, and HAST experiments (131 °C, 96% RH, 2.6bar, 96H) are then performed to test the corrosion resistance of the materials. The performance of the materials is shown as Table 4.

**Table 4 Corrosion resistance test results**

| Material components (at%, see the components in Embodiment 4) | Mass loss (mg/cm²) |
|---|---|
| Sintered NdFeB magnet rich in lanthanum and/or cerium | 89.31 |
| Sintered NdFeB magnet rich in lanthanum and/or cerium with addition of 4 wt% of alloy material rich in Co | 1.01 |

### Embodiment 5:

1, An NdFeB rare earth permanent magnet material rich in lanthanum and/or cerium and with components of Pr_{2.01}Nd_{5.88}Ce_{7.21}Ho_{0.4}Fe_{remaining}B_{6.21}M_{0.98} (at%) is prepared into an NdFeB rare earth permanent magnet material alloy rich in lanthanum and/or cerium by a quick-setting sheet process according to the technical scheme of the present invention;
2, An alloy material rich in Co and with components of Nd_{24.37}Pr_{8.31}Co_{60.02}Ga_{2.54}Nb_{4.76} (at%) is prepared by the quick-setting sheet process;
3, The NdFeB rare earth permanent magnet material alloy rich in lanthanum and/or cerium and the alloy material rich in Co are respectively subjected to hydrogen breaking, and are respectively subjected to jet milling powder preparation to obtain NdFeB rare earth permanent magnet material alloy powder rich in lanthanum and/or cerium and having an average particle diameter of 3.8 to 4.0 µm and alloy powder rich in Co and having an average particle diameter of 2.8 to 3.0 µm, the alloy powder rich in Co is added into the NdFeB rare earth permanent magnet material alloy powder rich in lanthanum and/or cerium at a ratio of 5wt%, and the two types of alloy powder are mixed uniformly by mixing;
4, The mixed powder is pressed and molded to form a square blank of 52 ^{∗} 52 ^{∗} 29 (mm) in an orientation magnetic field ≥1.6T;
5, The blank is placed into a high-vacuum sintering furnace for sintering at 1090 °C for 2.0 hours, first tempering at 900 °C for 2.5 hours and secondary tempering at 490 °C for 4.0 hours to obtain a sintered NdFeB magnet rich in lanthanum and/or cerium.
6, The obtained Pr_{2.01}Nd_{5.88}Ce_{7.21}Ho_{0.4}Fe_{remaining}B_{6.21}M_{0.98} (at%) NdFeB rare earth permanent magnet material alloy rich in lanthanum and/or cerium is directly prepared into a sintered NdFeB magnet rich in lanthanum and/or cerium without adding the alloy material rich in Co by using the same manufacturing process.

The two magnets are machined to prepare Φ10 ^{∗} 10 (mm) standard samples, and HAST experiments (131 °C, 96% RH, 2.6bar, 96H) are then performed to test the corrosion resistance of the materials. The performance of the materials is shown as Table 5.

**Table 5 Corrosion resistance test results**

| Material components (at%, see the components in Embodiment 5) | Mass loss (mg/cm²) |
|---|---|
| Sintered NdFeB magnet rich in lanthanum and/or cerium | 179.30 |
| Sintered NdFeB magnet rich in lanthanum and/or cerium with addition of 5 wt% of alloy material rich in Co | 0.98 |

## Claims

1. A corrosion-resistant sintered neodymium-iron-boron (NdFeB) magnet rich in lanthanum and/or cerium, comprising an NdFeB rare earth permanent magnet material rich in lanthanum and/or cerium and an alloy material rich in Co for improving the corrosion resistance of the material, wherein a component of the NdFeB rare earth permanent magnetic material rich in lanthanum and/or cerium is ReαFe100-α-β-γBβMγ, wherein Re is a rare earth element, consisting of two or more than two elements selected from La, Ce and Nd, and inevitably containing Nd element; wherein M is an additive element, consisting of one or more than one element selected from Ti, V, Cr, Ni, Zn, Ga, Ge, Al, Zr, Nb, Co, Cu, Ag, Sn, W, Pb, Bi and Pd; wherein Fe is Fe and unavoidable impurities; wherein α, β and γ are the atomic percentage contents of the elements, wherein 12≤α≤17, 5.1≤β≤6.8, and 0.1≤γ≤7.8; and wherein the alloy material rich in Co consists of two or more than two elements selected from Pr, Nd, Gd, Ho, Co, Ti, V, Zn, Ga, Al, Zr, Nb, Cu, Ag, Sn, Pb and Pd, and inevitably contains Co.

2. The corrosion-resistant sintered NdFeB magnet rich in lanthanum and/or cerium according to claim 1, **characterized in that** La and Ce elements in the rare-earth element Re account for 15 wt% to 45 wt% of total use amounts of rare earth in the NdFeB rare earth permanent magnet material rich in lanthanum and/or cerium.

3. The corrosion-resistant sintered NdFeB magnet rich in lanthanum and/or cerium according to claim 1, **characterized in that** the rare earth element Re further comprises one or more than one element selected from Pr, Pm, Sm, Eu, Gd, Ho, Er, Tm, Yb, Lu, Y and Sc.

4. The corrosion-resistant sintered NdFeB magnet rich in lanthanum and/or cerium according to claim 1, **characterized in that** the alloy material rich in Co inevitably does not contain element Fe.

5. A method of manufacturing a corrosion-resistant sintered NdFeB magnet rich in lanthanum and/or cerium, comprising the following specific operation steps:
(1) Preparing an NdFeB rare earth permanent magnet material alloy rich in lanthanum and/or cerium according to components of an NdFeB rare earth permanent magnet material rich in lanthanum and/or cerium of claim 1;
(2) Preparing an alloy material rich in Co according to components of the alloy material rich in Co of claim 1;
(3) Breaking the NdFeB rare earth permanent magnet material alloy rich in lanthanum and/or cerium to obtain NdFeB rare earth permanent magnet material alloy powder rich in lanthanum and/or cerium with an average particle size of 2.5 to 4.5 µm;
(4) Adding the alloy material rich in Co obtained in step (2) into the NdFeB rare earth permanent magnet material alloy powder rich in lanthanum and/or cerium according to a certain mass percentage content, wherein the process of pulverizing and mixing the alloy material rich in Co makes the alloy material rich in Co to be uniformly mixed into the NdFeB rare earth permanent magnet material alloy powder rich in lanthanum and/or cerium;
(5) Pressing and molding the mixed alloy powder into a blank in an oriented magnetic field ≥1.5T under the protection of a nitrogen atmosphere;
(6) Placing the molded blank in a high-vacuum sintering furnace for high-temperature sintering, and performing a two-stage tempering process to obtain the corrosion-resistant sintered NdFeB magnet rich in lanthanum and/or cerium.

6. A method of manufacturing a corrosion-resistant sintered NdFeB magnet rich in lanthanum and/or cerium according to claim 5, **characterized in that** a preparation process adopted in step (1) and step (2) is a casting process or a quick-setting sheet process; and in step (3), a breaking method adopted is mechanical breaking or hydrogen breaking plus jet milling.

7. A method of manufacturing a corrosion-resistant sintered NdFeB magnet rich in lanthanum and/or cerium according to claim 6, **characterized in that** the preparation process adopted in step (1) and step (2) is a quick-setting sheet process.

8. A method of manufacturing a corrosion-resistant sintered NdFeB magnet rich in lanthanum and/or cerium according to claim 7, **characterized in that** a roller speed of a cooling copper roller used in the quick-setting sheet process of step (2) is 5 to 15 times of a roller speed of a cooling copper roller used in the quick-setting sheet process of step (1).

9. A method of manufacturing a corrosion-resistant sintered NdFeB magnet rich in lanthanum and/or cerium according to claim 5, **characterized in that** in step (4), the mass percentage content of the alloy material rich in Co in the 1 NdFeB rare earth permanent magnet material alloy rich in lanthanum and/or cerium is 1% to 5%.

10. A method of manufacturing a corrosion-resistant sintered NdFeB magnet rich in lanthanum and/or cerium according to claim 5, **characterized in that** in step (6), sintering temperature is 1030 °C to 1090 °C, and sintering time is 2.0 to 8.0 hours, and a two-stage tempering process is that first tempering is carried out at 890 °C to 920, and constant temperature time is 1.5 to 3 hours; and secondary tempering is carried out at 480 °C to 520 °C, and constant temperature time is 2 to 6 hours.

## Patentansprüche

1. Ein korrosionsbeständiger gesinterter lanthan- und/oder cerreicher Neodym-Eisen-Bor-Magnet (NdFeB), umfassend ein NdFeB-Seltenerd-Permanentmagnet-Material, das reich an Lanthan und/oder Cer ist, und ein Legierungsmaterial, das reich an Co ist, zur Verbesserung der Korrosionsbeständigkeit des Materials, wobei eine Komponente des NdFeB-Seltenerd-Permanentmagnet-Materials, das reich an Lanthan und/oder Cer ist, ReαFelOO-α-β-γBβMγ ist, wobei Re ein Seltenerdelement ist, das aus zwei oder mehr als zwei Elementen besteht,
ausgewählt aus La, Ce und Nd, und zwangsläufig das Element Nd enthalten; wobei M ein Zusatzelement ist, bestehend aus einem oder mehr als einem Element, ausgewählt aus Ti, V, Cr, Ni, Zn, Ga, Ge, Al, Zr, Nb, Co, Cu, Ag, Sn, W, Pb, Bi und Pd; wobei Fe Fe und unvermeidbare Verunreinigungen ist; wobei α, β und γ die atomaren Prozentgehalte der Elemente sind, wobei 12≤α≤17, 5,1≤β≤6,8, und 0,1≤γ≤7,8; und wobei das Co-reiche Legierungsmaterial aus zwei oder mehr als zwei Elementen besteht, ausgewählt aus Pr, Nd, Gd, Ho, Co, Ti, V, Zn, Ga, Al, Zr, Nb, Cu, Ag, Sn, Pb und Pd, und die zwangsläufig Co enthalten.

2. Der korrosionsbeständige gesinterte lanthan- und/oder cerreiche NdFeB-Magnet nach Anspruch 1, **dadurch gekennzeichnet, dass** die La- und Ce-Elemente im Seltenerdelement Re 15 Gew.-% bis 45 Gew.-% der gesamten Einsatzmengen an Seltenerde im lanthan- und/oder cerreichen NdFeB-Seltenerd-Permanentmagnet-Material ausmachen.

3. Der korrosionsbeständige gesinterte lanthan- und/oder cerreiche NdFeB-Magnet nach Anspruch 1, **dadurch gekennzeichnet, dass** das Seltenerdelement Re ferner ein oder mehr als ein Element umfasst, das aus Pr, Pm, Sm, Eu, Gd, Ho, Er, Tm, Yb, Lu, Y und Sc ausgewählt ist.

4. Der korrosionsbeständige gesinterte lanthan- und/oder cerreiche NdFeB-Magnet nach Anspruch 1, **dadurch gekennzeichnet, dass** das co-reiche Legierungsmaterial zwangsläufig kein Element Fe enthält.

5. Ein Verfahren zur Herstellung eines korrosionsbeständigen gesinterten lanthan- und/oder cerreichen NdFeB-Magneten, umfassend die folgenden spezifischen Arbeitsschritte:
(1) Herstellen einer lanthan- und/oder cerreichen NdFeB-Seltenerd-Permanentmagnet-Materiallegierung, gemäß Komponenten eines lanthan- und/oder cerreichen NdFeB-Seltenerd-Permanentmagnet-Materials nach Anspruch 1,
(2) Herstellen eines Co-reichen Legierungsmaterials gemäß Komponenten des Co-reichen Legierungsmaterials nach Anspruch 1,
(3) Brechen der lanthan- und/oder cerreichen NdFeB-Seltenerd-Permanentmagnet-Materiallegierung, um lanthan- und/oder cerreiches NdFeB-Seltenerd-Permanentmagnet-Material-Legierungspulver mit einer durchschnittlichen Partikelgröße von 2,5 bis 4,5 pm zu erhalten;
(4) Hinzufügen des in Schritt (2) erhaltenen co-reichen Legierungsmaterials zu dem lanthan- und/oder cerreichen Legierungspulver aus dem NdFeB-Seltenerd-Permanentmagnet-Material gemäß einem bestimmten prozentualen Massenanteil, wobei der Prozess des Pulverisierens und Mischens des co-reichen Legierungsmaterials das co-reiche Legierungsmaterial dazu bringt, gleichmäßig in das lanthan- und/oder cerreiche Legierungspulver aus dem NdFeB-Seltenerd-Permanentmagnet-Material gemischt zu werden;
(5) Pressen und Formen des gemischten Legierungspulvers zu einem Rohling in einem orientierten Magnetfeld ≥1,5 T unter dem Schutz einer Stickstoffatmosphäre;
(6) Platzieren des geformten Rohlings in einem Hochvakuumsinterofen zum Hochtemperatursintern und Durchführen eines zweistufigen Temperprozesses, um den korrosionsbeständigen gesinterten lanthan- und/oder cerreichen NdFeB-Magneten zu erhalten.

6. Ein Verfahren zur Herstellung eines korrosionsbeständigen gesinterten lanthan- und/oder cerreichen NdFeB-Magneten nach Anspruch 5, **dadurch gekennzeichnet, dass** ein in Schritt (1) und Schritt (2) angewendetes Herstellungsverfahren ein Gießverfahren oder ein schnell abbindendes Folienverfahren ist; und in Schritt (3) ein angewendetes Brechverfahren mechanisches Brechen oder Wasserstoffbrechen plus Strahlmahlen ist.

7. Ein Verfahren zur Herstellung eines korrosionsbeständigen gesinterten lanthan- und/oder cerreichen NdFeB-Magneten nach Anspruch 6, **dadurch gekennzeichnet, dass** der in Schritt (1) und Schritt (2) angewandte Herstellungsprozess ein schnell abbindender Folienprozess ist.

8. Ein Verfahren zur Herstellung eines korrosionsbeständigen gesinterten lanthan- und/oder cerreichen NdFeB-Magneten nach Anspruch 7, **dadurch gekennzeichnet, dass** die Walzendrehzahl einer Kühlkupferwalze, die in dem schnell abbindenden Blechprozess von Schritt (2) verwendet wird, das 5- bis 15-fache der Walzendrehzahl einer Kühlkupferwalze beträgt, die in dem schnell abbindenden Blechprozess von Schritt (1) verwendet wird.

9. Ein Verfahren zur Herstellung eines korrosionsbeständigen gesinterten lanthan- und/oder cerreichen NdFeB-Magneten nach Anspruch 5, **dadurch gekennzeichnet, dass** in Schritt (4) der prozentuale Massenanteil des Co-reichen Legierungsmaterials an dem einen lanthan- und/oder cerreichen NdFeB-Seltenerd-Permanentmagnet-Materials 1 % bis 5 % beträgt.

10. Ein Verfahren zur Herstellung eines korrosionsbeständigen gesinterten lanthan- und/oder cerreichen NdFeB-Magneten nach Anspruch 5, **dadurch gekennzeichnet, dass** in Schritt (6) die Sintertemperatur 1030 °C bis 1090 °C beträgt und die Sinterzeit 2,0 bis 8,0 Stunden beträgt, und ein zweistufiges Temperverfahren darin besteht, dass das erste Tempern bei 890 °C bis 920 °C durchgeführt wird und die konstante Temperaturzeit 1,5 bis 3 Stunden beträgt; und das zweite Tempern bei 480 °C bis 520 °C durchgeführt wird und die konstante Temperaturzeit 2 bis 6 Stunden beträgt.

## Revendications

1. Aimant en néodyme-fer-bore (NdFeB) fritté résistant à la corrosion, riche en lanthane et/ou en cérium, comprenant un matériau d'aimant permanent en terre rare NdFeB riche en lanthane et/ou en cérium et un matériau d'alliage riche en Co pour améliorer la résistance à la corrosion du matériau, dans lequel un composant du matériau d'aimant permanent en terre rare NdFeB riche en lanthane et/ou en cérium est ReαFe100-α-β-γBβMγ, où Re est un élément de terre rare, constitué de deux éléments ou plus sélectionné parmi La, Ce et Nd, et contenant inévitablement un élément Nd ; où M est un élément additif, constitué d'un ou plusieurs éléments sélectionnés parmi Ti, V, Cr, Ni, Zn, Ga, Ge, Al, Zr, Nb, Co, Cu, Ag, Sn, W, Pb, Bi et Pd ; où Fe est Fe et des impuretés inévitables ; où α, β et γ sont les teneurs en pourcentage atomique des éléments, où 12≤α≤17, 5.1≤β≤6.8, et 0.1≤γ≤7.8 ; et dans lequel le matériau d'alliage riche en Co est constitué de deux ou plus de deux éléments sélectionnés parmi Pr, Nd, Gd, Ho, Co, Ti, V, Zn, Ga, Al, Zr, Nb, Cu, Ag, Sn, Pb et Pd, et contient inévitablement Co.

2. L'Aimant NdFeB fritté résistant à la corrosion riche en lanthane et/ou en cérium selon la revendication 1, **caractérisé en ce que** les éléments La et Ce dans l'élément de terre rare Re représentent de 15% en poids à 45% en poids des quantités totales utilisées de terre rare dans le matériau d'aimant permanent de terre rare NdFeB riche en lanthane et/ou en cérium.

3. L'Aimant NdFeB fritté résistant à la corrosion riche en lanthane et/ou en cérium selon la revendication 1, **caractérisé en ce que** l'élément de terre rare Re comprend en outre un ou plusieurs éléments choisis parmi Pr, Pm, Sm, Eu, Gd, Ho, Er, Tm, Yb, Lu, Y et Sc.

4. L'Aimant NdFeB fritté résistant à la corrosion, riche en lanthane et/ou en cérium selon la revendication 1, **caractérisé en ce que** le matériau d'alliage riche en Co inévitablement ne contient pas d'élément Fe.

5. Procédé de fabrication d'un aimant NdFeB fritté résistant à la corrosion, riche en lanthane et/ou en cérium, comprenant les étapes opératoires spécifiques suivantes :
(1) Préparer un alliage de matériau d'aimant permanent de terre rare NdFeB riche en lanthane et/ou en cérium selon des composants d'un matériau d'aimant permanent de terre rare NdFeB riche en lanthane et/ou en cérium de la revendication 1 ;
(2) Préparer un matériau d'alliage riche en Co selon les composants du matériau d'alliage riche en Co de la revendication 1 ;
(3) Briser l'alliage de matériau d'aimant permanent de terre rare NdFeB riche en lanthane et/ou en cérium pour obtenir une poudre d'alliage de matériau d'aimant permanent de terre rare NdFeB riche en lanthane et/ou en cérium avec une granulométrie moyenne de 2,5 à 4,5 µm ;
(4) Ajouter le matériau d'alliage riche en Co obtenu à l'étape (2) dans la poudre d'alliage de matériau d'aimant permanent de terre rare NdFeB riche en lanthane et/ou en cérium selon une certaine teneur en pourcentage en masse, dans lequel le processus de pulvérisation et de mélange du matériau d'alliage riche en Co rend le matériau d'alliage riche en Co à mélanger uniformément dans la poudre d'alliage de matériau d'aimant permanent de terre rare NdFeB riche en lanthane et/ou en cérium ;
(5) Presser et mouler la poudre d'alliage mélangée en une ébauche dans un champ magnétique orienté ≥1,5T sous la protection d'une atmosphère d'azote ;
(6) Placer l'ébauche moulée dans un four de frittage sous vide poussé pour frittage à haute température, et effectuer un processus de revenu en deux étapes pour obtenir l'aimant NdFeB fritté résistant à la corrosion riche en lanthane et/ou en cérium.

6. Procédé de fabrication d'un aimant NdFeB fritté résistant à la corrosion riche en lanthane et/ou en cérium selon la revendication 5, **caractérisé en ce qu'**un procédé de préparation adopté à l'étape (1) et à l'étape (2) est un procédé de coulée ou un procédé à feuille à prise rapide ; et à l'étape (3), un procédé de rupture adopté est une rupture mécanique ou une rupture à l'hydrogène plus un broyage par jet.

7. Procédé de fabrication d'un aimant NdFeB fritté résistant à la corrosion riche en lanthane et/ou en cérium selon la revendication 6, **caractérisé en ce que** le procédé de préparation adopté dans les étapes (1) et (2) est un procédé à feuille à prise rapide.

8. Procédé de fabrication d'un aimant NdFeB fritté résistant à la corrosion, riche en lanthane et/ou en cérium selon la revendication 7, **caractérisé en ce que** la vitesse de rotation d'un rouleau de cuivre de refroidissement utilisé dans le processus de feuille à prise rapide de l'étape (2) est de 5 à 15 fois la vitesse de rotation d'un rouleau de cuivre de refroidissement utilisé dans le processus de feuille à prise rapide de l'étape (1).

9. Procédé de fabrication d'un aimant NdFeB fritté résistant à la corrosion riche en lanthane et/ou en cérium selon la revendication 5, **caractérisé en ce que** dans l'étape (4), la teneur en pourcentage massique du matériau d'alliage riche en Co dans l'alliage de matériau d'aimant permanent de terre rare 1 NdFeB riche en lanthane et/ou en cérium est de 1% à 5%.

10. Procédé de fabrication d'un aimant NdFeB fritté résistant à la corrosion riche en lanthane et/ou en cérium selon la revendication 5, **caractérisé en ce que** dans l'étape (6), la température de frittage est de 1030°C à 1090°C, et le temps de frittage est de 2,0 à 8,0 heures, et un procédé de revenu en deux étapes est que le premier revenu est effectué à 890°C jusqu'à 920, et le temps de température constante est de 1,5 à 3 heures ; et le revenu secondaire est effectué à 480°C jusqu'à 520°C, et le temps de température constante est de 2 à 6 heures.
